

# United States Patent

[19]

Habu et al.

[11]

4,318,979

[45]

Mar. 9, 1982

[54] **LIGHT-SENSITIVE SILVER HALIDE  
PHOTOGRAPHIC MATERIAL**

[75] Inventors: **Takeshi Habu; Chika Honda**, both of  
Hino, Japan

[73] Assignee: **Konishiroku Photo Industry Co., Ltd.**,  
Tokyo, Japan

[21] Appl. No.: **215,011**

[22] Filed: **Dec. 10, 1980**

## Related U.S. Application Data

[63] Continuation of Ser. No. 70,846, Aug. 29, 1979, abandoned.

## Foreign Application Priority Data

Sep. 7, 1978 [JP] Japan ..... 53-109910

[51] Int. Cl.<sup>3</sup> ..... G03C 1/06; G03C 5/24

[52] U.S. Cl. ..... 430/434; 430/436;  
430/437; 430/439; 430/438; 430/440; 430/442;  
430/141; 430/170; 430/564; 430/614; 430/612;  
430/600; 430/949

[58] **Field of Search** ..... 430/434, 436, 437, 439,  
430/438, 440, 442, 170, 141, 564, 614, 949, 600,  
612, 149

[56]

## References Cited

### U.S. PATENT DOCUMENTS

|           |         |                |       |         |
|-----------|---------|----------------|-------|---------|
| 2,839,405 | 6/1958  | Jones          | ..... | 430/608 |
| 3,488,709 | 1/1970  | Sidebotham     | ..... | 430/608 |
| 3,556,797 | 1/1971  | Pattijn et al. | ..... | 430/612 |
| 3,891,442 | 6/1975  | Beavers        | ..... | 430/564 |
| 3,901,712 | 8/1975  | Beavers        | ..... | 430/564 |
| 4,169,733 | 10/1979 | Iytaka et al.  | ..... | 430/949 |

## OTHER PUBLICATIONS

Derwent Abstract: 09348 Y/06, E 19 G06, 02-08-1975,  
JA-094295 (02-02-77).

Primary Examiner—Won H. Louie, Jr.

Attorney, Agent, or Firm—Frishauf, Holtz, Goodman &  
Woodward

[57]

## ABSTRACT

A light-sensitive silver halide photographic material comprising a combination of a salt of tetrazolium containing only a non-metallic anion and a salt of tetrazolium containing a metallic anion.

10 Claims, No Drawings

LIGHT-SENSITIVE SILVER HALIDE  
PHOTOGRAPHIC MATERIAL

This is a continuation of application Ser. No. 70,846 filed Aug. 29, 1979, now abandoned.

This invention relates to a novel light-sensitive silver halide photographic material and particularly to a novel lith-type light-sensitive silver halide photographic material for obtaining a photographic image with especially high contrast, high sharpness and high resolving power.

More particularly, this invention relates to a high-contrast light-sensitive silver halide photographic material that is advantageously employed for forming a line- or dot-image. Accordingly, this invention relates particularly to a lith-type light-sensitive silver halide photographic material for printing and to a light-sensitive material for copying.

A high-contrast photographic characteristic bringing about only maximum and minimum concentration portions (so-called fringe) is necessary for obtaining a dot- or line image required in the printing processes.

For the purpose of forming such a photographic image as stated above, a process involving the combination of a high-contrast light-sensitive photographic material and a developer (lith-type developer) capable of developing said material infectiously is known.

As for said lith-type developer, there is a detailed description in J.A.C. Yule, Journal of the Franklin Institute, vol. 239, page 221 (1945).

The lith-type developer, however, is poor in maintaining its activity during storage. Therefore, a plate maker is required to control the developer for maintaining the activity of the developer, which changes on standing, at a constant level in order to obtain a halftone negative or halftone positive image with high quality. The control required in the above-mentioned process involves disadvantageously complicated procedures and, if the automatic procedures are adopted, they should require uneconomical expense.

The lith-type developer contains inherently the low-concentration of the sulfite ion and also contains inherently the relatively high concentration of the hydroquinone developing agent in an aqueous alkaline solution, so that automatic oxidation is apt to take place. This is the reason why the lith-type developer is poor in storage stability.

Many proposals on the improvement of the storage 50 stability have been previously made. One of the proposals suggests that a light-sensitive silver halide photographic material containing a tetrazolium compound which yields a high contrast silver image even when the photographic material be developed by a so-called PQ-type or MQ-type conventional developer (e.g., a developer based on the Phenidone (R)/Hydroquinone or Metol (R)/Hydroquinone mixture as developing agents, respectively) having the sufficiently high concentration of the sulfite ion, as disclosed, for instance, by Japanese Patent Provisional Publication 52(1977)-18,317. By the addition of the tetrazolium compound, the photographic material can be developed in a conventional developer that has excellent storage stability. Nevertheless, the light-sensitive silver halide photographic material containing the tetrazolium compound is, on the contrary, poor in storage stability, that is, said photographic material yields a dot-image whose contrast

lowers when it was stored for long time at room temperature before exposure.

Accordingly, it is the primary object of the invention to provide a light-sensitive silver halide photographic material that can yield a black-and-white silver image, particularly a dot- or line-image, with high contrast even when developed in a stable developer and that has sufficient storage stability. Other objects of the invention are apparent from the description set forth herein-after.

As a result of the study, the present inventors have found that the objects can be accomplished by incorporating the combination of a salt of tetrazolium containing only a non-metallic anion and a salt of tetrazolium containing a metallic anion into a light-sensitive silver halide photographic material.

The salt of tetrazolium containing only a non-metallic anion has Formula (I), and the salt of tetrazolium containing a metallic anion has Formula (II):



In the above formulae, T represents a tetrazolium cation,  $X_1$  represents an anion containing only non-metallic atoms,  $X_2$  represents an anion containing a metal atom, n is 1 or 2, m is an integer of 1 to 3, and  $m_1$  is an integer yielding that n multiplied by  $m_1$  is equal to m.

In formula (I), T has the formula (I-a), (I-b) or (I-c).



In formulae (I-a), (I-b) and (I-c),  $R_1$ ,  $R_2$ ,  $R_3$ ,  $R_4$ ,  $R_5$ ,  $R_6$ ,  $R_7$ ,  $R_8$ ,  $R_9$ ,  $R_{10}$  and  $R_{11}$ , which may be the same or different, are hydrogen or halogen atoms, amino, nitro, cyano, mercapto, hydroxy, carboxy, alkyl, alkenyl, alkoxy, alkoxy carbonyl, aryl, acyl or heterocyclic groups, or groups that are capable of forming metallic chelate compounds or complex compounds. The last groups set forth in the above sentence are ones that act as electron donor to form coordination compounds with metal ions, and are exemplified by pyridyl and dipyridyl groups. The above-listed amino, alkyl, alkenyl, alkoxy, alkoxy carbonyl, aryl and heterocyclic groups can have one or more substituents, such as halogen, amino, nitro, cyano, mercapto, alkyl, hydroxy, alkenyl, alkoxy carbonyl, aryl or a hetero-cyclic group.

In these formulae, D and E, which may be the same or different, are arylene groups such as phenylene and naphthylene, or alkylene groups, preferably having 1 to

18 carbon atoms, such as methylene, octamethylene, propylene, butylene and octadecylene. These arylene and alkylene groups can have one or more substituents, such as amino, nitro, cyano, mercapto, hydroxy, carboxy, alkyl, alkenyl, alkoxy carbonyl, aryl or a heterocyclic group.

In these formulae (I-a), (I-b) and (I-c), the alkyl group preferably contains 1 to 32 carbon atoms and its examples include methyl, butyl, octyl, octadecyl and eicosyl; the alkenyl group preferably contains 2 to 20 carbon atoms and its example includes allyl, butenyl, octenyl or octadecyl; the aryl group preferably is phenyl or naphthyl group including, for example, phenyl, hydroxyphenyl, aminophenyl, carboxyphenyl, nitrophenyl, alkylphenyl, sulfophenyl, alfa-naphthyl, beta-naphthyl, hydroxynaphthyl, carboxynaphthyl and aminonaphthyl; the alkoxy group preferably contains 1 to 32 carbon atoms including, for example, methoxy, ethoxy and octadecyloxy; and the alkoxy carboxy group preferably contains 2 to 32 carbon atoms including, for example, methoxycarbonyl, ethoxycarbonyl and octadecyloxy. Example of the heterocyclic group includes oxazolyl, thiazolyl, imidazolyl, benzoxazolyl, benzthiazolyl, benzimidazolyl, selenazolyl, benzelenazolyl, quinonyl, quinazolyl, triazolyl, naphthoxazolyl, pyridyl, pyrimidyl, indazolyl, furyl, oxadiazolyl, thienylmorpholino, piperidyl and tetrazolyl, and the heterocyclic group preferably is a five or six-membered heterocyclic group or condensed heterocyclic group containing nitrogen, oxygen and/or sulfur atoms. The halogen atom is, for instance, a chlorine, bromine or iodine atom.

In the formulae (I-a), (I-b) and (I-c), particularly preferred groups for R<sub>1</sub>, R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>10</sub> and R<sub>11</sub> are substituted or unsubstituted aryl groups.

Among the groups of the formulae identified above, the most preferred is a group represented by the formula (I-a) followed by a group represented by the formula (I-b) which is further followed by a group represented by the formula (I-c). The utmost preferred group is a group represented by the formula (I-a) in which R<sub>1</sub>, R<sub>2</sub> and R<sub>3</sub> are the substituted or unsubstituted phenyl groups.

X<sub>1</sub> represents an anionic atom or group containing only non-metallic atoms and is exemplified by a halogen atom and groups of the formulae (I-d), (I-e), (I-f), (I-g) and (I-h).



Formula (I-d)

In Formula (I-d), R<sub>12</sub> represents an alkyl group preferably containing 14 to 32 carbon atoms, whose example includes tetradecyl, hexadecyl and octadecyl. Said alkyl can be substituted by an optional substituent, for example, a halogen atom such as a chlorine or bromine atom. Alternatively, R<sub>12</sub> represents a group of the formula:



in which R<sub>13</sub> and R<sub>14</sub>, which may be the same or different, represent hydrogen, halogen such as chlorine or

bromine, alkyl such as methyl, ethyl or butyl or phenyl, said alkyl and phenyl being optionally substituted by alkyl (e.g., methyl, ethyl, propyl, isopropyl or butyl) or halogen (e.g., chlorine or bromine). n<sub>1</sub> is an integer of 1 to 3. n<sub>2</sub> is an integer of 1 to 20.



In the formulae (I-e) and (I-f), R<sub>14</sub>, R<sub>15</sub>, R<sub>16</sub>, R<sub>17</sub> and R<sub>18</sub>, may be the same or different. Each of them represents a halogen atom such as chlorine or bromine atom, or an alkyl group containing preferably 1 to 32 carbon atoms, whose example includes, a methyl, ethyl, butyl, isobutyl, pentyl, hexyl, octyl, nonyl, decyl or dodecyl or octadecyl group. Said alkyl group can be substituted by halogen such as chlorine or bromine or aryl such as phenyl or naphthyl. R<sub>19</sub> and R<sub>20</sub>, which may be the same or different, are carboxy, sulfo or phosphoric acid groups.



Formula (I-g)

In formula (I-g), R<sub>21</sub> and R<sub>22</sub>, which may be the same or different, represent a hydrogen or halogen atom, or an alkyl or alkenyl group containing preferably 1 to 18 carbon atoms, for example, methyl, ethyl, butyl, isobutyl, octyl, allyl, butenyl and octenyl. n<sub>3</sub>, n<sub>4</sub> and n<sub>5</sub>, which may be the same or different, are integers of 1 to 3.



Formula (I-h)

In Formula (I-h), Y represents a sulfur, selenium, oxygen or nitrogen atom or a divalent residual group of the formula—NR<sub>24</sub>—in which R<sub>24</sub> is hydrogen, alkyl or aryl. Z represents an atomic group required for completing a five- or six-membered hetero-ring containing oxygen, selenium or nitrogen as a hetero atom, such as a thiazole, selenazole, oxazole, imidazole, pyrazole, triazole, tetrazole, pyrimidine or triazine ring. On the carbon atoms of said hetero-ring, there can be placed a variety of substituents, for instance, alkyl containing 1 to 20 carbon atoms, such as, methyl, ethyl, n-butyl, heptyl or octadecyl, alkoxy containing 1 to 20 carbon atoms, such as, methoxy, ethoxy, dodecyl, heptadecyloxy, alkylthio containing 1 to 20 carbon atoms, such as, methylthio, ethylthio or butylthio. R<sub>23</sub> has the same meaning as R<sub>22</sub>. n<sub>6</sub> is 1 or 2.

Examples of the group T and the anion X<sub>1</sub><sup>⊖</sup> of Formula (I) representing the compound employed in this invention are listed below, but these examples are not intended to limit this invention.

-continued

| Examples for T |                                                                                                | Examples for $X_1$    |                                                                                                                                                           |
|----------------|------------------------------------------------------------------------------------------------|-----------------------|-----------------------------------------------------------------------------------------------------------------------------------------------------------|
| T - (1)        | 2-(Benzothiazol-2-yl)-3-phenyl-5-dodecyl-2H-tetrazolium                                        | X <sub>1</sub> - (4)  | $\text{CH}_3(\text{CH}_2)_{11}-\text{C}_6\text{H}_4-\text{SO}_3^-$                                                                                        |
| T - (2)        | 2,3-Diphenyl-5-(4-t-oxyloxyphenyl)-2H-tetrazolium                                              | 5                     | $\text{CH}_3(\text{CH}_2)_{17}-\text{C}_6\text{H}_4-\text{SO}_3^-$                                                                                        |
| T - (3)        | 2,3,5-Triphenyl-2H-tetrazolium                                                                 | X <sub>1</sub> - (5)  |                                                                                                                                                           |
| T - (4)        | 2,3,5-Tri(p-carboxyethylphenyl)-2H-tetrazolium                                                 | 10                    | $\text{CH}_3(\text{CH}_2)_{17}-\text{C}_6\text{H}_4-\text{SO}_3^-$                                                                                        |
| T - (5)        | 2-(Benzothiazol-2-yl)-3-phenyl-5-(o-chlorophenyl)-2H-tetrazolium                               | X <sub>1</sub> - (6)  | $\text{CH}_3-\overset{\text{CH}_3}{\underset{\text{CH}_3}{\text{CH}}}(\text{CH}_2)-\text{CH}_2-\text{CH}(\text{CH}_3)-\text{C}_6\text{H}_4-\text{SO}_3^-$ |
| T - (6)        | 2,3-Diphenyl-2H-tetrazolium                                                                    | 15                    |                                                                                                                                                           |
| T - (7)        | 2,3-Diphenyl-5-methyl-2H-tetrazolium                                                           | X <sub>1</sub> - (7)  | $\text{CH}_3(\text{CH}_2)_{11}-\text{C}_6\text{H}_4-\text{SO}_3^-$                                                                                        |
| T - (8)        | 3-(p-Hydroxyphenyl)-5-methyl-2-phenyl-2H-tetrazolium                                           | 20                    | $\text{CH}_3(\text{CH}_2)_{11}-\text{C}_6\text{H}_4-\text{SO}_3^-$                                                                                        |
| T - (9)        | 2,3-Diphenyl-5-ethyl-2H-tetrazolium                                                            | X <sub>1</sub> - (8)  | $\text{CH}_3(\text{CH}_2)_{11}-\text{C}_6\text{H}_4-\text{SO}_3^-$                                                                                        |
| T - (10)       | 2,3-Diphenyl-5-n-hexyl-2H-tetrazolium                                                          | 25                    | $\text{CH}_3(\text{CH}_2)_{11}-\text{C}_6\text{H}_4-(\text{CH}_2)_{11}\text{CH}_3$                                                                        |
| T - (11)       | 5-Cyano-2,3-diphenyl-2H-tetrazolium                                                            | X <sub>1</sub> - (9)  |                                                                                                                                                           |
| T - (12)       | 2-(Benzothiazol-2-yl)-5-phenyl-3-(4-tolyl)-2H-tetrazolium                                      | 30                    | $\text{CH}_3(\text{CH}_2)_{17}-\text{C}_6\text{H}_4-(\text{CH}_2)_4\text{CH}_3$                                                                           |
| T - (13)       | 2-(Benzothiazol-2-yl)-5-(4-chlorophenyl)-3-(4-nitrophenyl)-2H-tetrazolium                      | X <sub>1</sub> - (10) |                                                                                                                                                           |
| T - (14)       | 5-Ethoxycarbonyl-2,3-di(3-nitrophenyl)-2H-tetrazolium                                          | 35                    | $\text{CH}_3-\text{C}(\text{CH}_3)_2-\text{CH}_2-\text{CH}(\text{CH}_3)-\text{CH}_2\text{OOC}-\text{CH}_2$                                                |
| T - (15)       | 5-Acetyl-2,3-di(p-ethoxyphenyl)-2H-tetrazolium                                                 | X <sub>1</sub> - (11) | $\text{CH}_3-\text{C}(\text{CH}_3)_2-\text{CH}_2-\text{CH}(\text{CH}_3)-\text{CH}_2\text{OOC}-\text{CH}-\text{SO}_3^-$                                    |
| T - (16)       | 2,5-Diphenyl-3-(p-tolyl)-2H-tetrazolium                                                        | X <sub>1</sub> - (12) | $\text{CH}_3(\text{CH}_2)_{11}-\text{OOC}-\text{CH}_2$                                                                                                    |
| T - (17)       | 2,5-Diphenyl-3-(p-iodophenyl)-2H-tetrazolium                                                   | 40                    | $\text{CH}_3(\text{CH}_2)_{17}\text{OOC}-\text{CH}_2$                                                                                                     |
| T - (18)       | 2,3-Diphenyl-5-(p-diphenyl)-2H-tetrazolium                                                     | X <sub>1</sub> - (13) | $\text{CH}_3(\text{CH}_2)_{17}\text{OOC}-\text{CH}-\text{SO}_3^-$                                                                                         |
| T - (19)       | 5-(p-Bromophenyl)-2-phenyl-3-(2,4,6-trichlorophenyl)-2H-tetrazolium                            | 45                    | $\text{CH}_3(\text{CH}_2)_5-\text{OOC}-\text{CH}_2$                                                                                                       |
| T - (20)       | 3-(p-Hydroxyphenyl)-5-(p-nitrophenyl)-2-phenyl-2H-tetrazolium                                  | X <sub>1</sub> - (14) | $\text{CH}_3(\text{CH}_2)_5-\text{OOC}-\text{CH}-\text{SO}_3^-$                                                                                           |
| T - (21)       | 5-(3,4-Dimethoxyphenyl)-3-(2-ethoxyphenyl)-2-(4-methoxyphenyl)-2H-tetrazolium                  | 50                    | $\text{CH}_3(\text{CH}_2)_8-\text{OOC}-\text{CH}_2$                                                                                                       |
| T - (22)       | 5-(4-Cyanophenyl)-2,3-diphenyl-2H-tetrazolium                                                  | X <sub>1</sub> - (15) | $\text{CH}_3(\text{CH}_2)_4-\text{OOC}-\text{CH}-\text{SO}_3^-$                                                                                           |
| T - (23)       | 3-(p-Acetamidophenyl)-2,5-diphenyl-2H-tetrazolium                                              | 55                    | $\text{C}_6\text{H}_5-\text{OCOCH}_2$                                                                                                                     |
| T - (24)       | 5-Acetyl-2,3-diphenyl-2H-tetrazolium                                                           | X <sub>1</sub> - (16) | $\text{C}_6\text{H}_5-\text{OCOCH}-\text{SO}_3^-$                                                                                                         |
| T - (25)       | 5-(Fur-2-yl)-2,3-diphenyl-2H-tetrazolium                                                       | 60                    | $\text{C}_6\text{H}_5-\text{OCOCH}_2$                                                                                                                     |
| T - (26)       | 5-(Thien-2-yl)-2,3-diphenyl-2H-tetrazolium                                                     | X <sub>1</sub> - (17) | $\text{C}_6\text{H}_5-\text{OCOCH}-\text{COO}^-$                                                                                                          |
| T - (27)       | 2,3-Diphenyl-5-(pyrido-4-yl)-2H-tetrazolium                                                    | 65                    | $\text{CH}_3(\text{CH}_2)_2-\text{C}_6\text{H}_4-\text{OCOCH}_2$                                                                                          |
| T - (28)       | 2,3-Diphenyl-5-(quinol-2-yl)-2H-tetrazolium                                                    | X <sub>1</sub> - (18) | $\text{CH}_3(\text{CH}_2)_2-\text{C}_6\text{H}_4-\text{OCOCH}-\text{SO}_3^-$                                                                              |
| T - (29)       | 2,3-Diphenyl-5-(benzoxazol-2-yl)-2H-tetrazolium                                                |                       |                                                                                                                                                           |
| T - (30)       | 2,3-Diphenyl-5-nitro-2H-tetrazolium                                                            |                       |                                                                                                                                                           |
| T - (31)       | 2,2',3,3'-Tetraphenyl-5,5'-1,4-butenyl-di-(2H-tetrazolium)                                     |                       |                                                                                                                                                           |
| T - (32)       | 2,2',3,3'-Tetraphenyl-5,5'-p-phenylen-di-(2H-tetrazolium)                                      |                       |                                                                                                                                                           |
| T - (33)       | 2-(4,5-Dimethylthiazol-2-yl)-3,5-diphenyl-2H-tetrazolium                                       |                       |                                                                                                                                                           |
| T - (34)       | 3,5-Diphenyl-2-(triazin-2-yl)-2H-tetrazolium                                                   |                       |                                                                                                                                                           |
| T - (35)       | 2-(Benzothiazol-2-yl)-3-(4-methoxyphenyl)-5-phenyl-2H-tetrazolium                              |                       |                                                                                                                                                           |
| T - (36)       | 3,3'-(3,3'-Dimethoxy-4,4'-biphenyl)-bis[2-(p-nitrophenyl)-5-phenyl-2H-tetrazolium]             |                       |                                                                                                                                                           |
| T - (37)       | 3,3'-(3,3'-Dimethoxy-4,4'-biphenyl)-bis(p-nitrophenyl)-5-(p-thiocarbamylphenyl)-2H-tetrazolium |                       |                                                                                                                                                           |
| T - (38)       | 3,3'-(3,3'-Dimethoxy-4,4'-biphenyl)-bis[2,5-bis(p-nitrophenyl)-2H-tetrazolium]                 |                       |                                                                                                                                                           |
| T - (39)       | 3,3'-(3,3'-Dimethoxy-4,4'-biphenyl)-bis[2,5-diphenyl-2H-tetrazolium]                           |                       |                                                                                                                                                           |
| T - (40)       | 2,5-Diphenyl-3- $\beta$ -naphthyltetrazolium                                                   |                       |                                                                                                                                                           |
| T - (41)       | 2-p-Iodophenyl-3-p-nitrophenyl-5-phenyl-2H-tetrazolium                                         |                       |                                                                                                                                                           |

| Examples for $X_1$    |                                                                                                                                                                                        |
|-----------------------|----------------------------------------------------------------------------------------------------------------------------------------------------------------------------------------|
| X <sub>1</sub> - (1)  | $\text{CH}_3-\overset{\text{CH}_3}{\underset{\text{CH}_3}{\text{C}}}(\text{CH}_2)-\overset{\text{CH}_3}{\underset{\text{H}}{\text{C}}}-\text{CH}_2-\text{C}_6\text{H}_4-\text{SO}_3^-$ |
| X <sub>1</sub> - (2)  | $\text{CH}_3-\overset{\text{CH}_3}{\underset{\text{CH}_3}{\text{C}}}(\text{CH}_2)-\text{C}_6\text{H}_4-\text{SO}_3^-$                                                                  |
| X <sub>1</sub> - (3)  | $\text{CH}_3-\overset{\text{H}}{\underset{\text{CH}_3}{\text{C}}}(\text{CH}_2)-\text{C}_6\text{H}_4-\text{SO}_3^-$                                                                     |
| X <sub>1</sub> - (4)  |                                                                                                                                                                                        |
| X <sub>1</sub> - (5)  |                                                                                                                                                                                        |
| X <sub>1</sub> - (6)  |                                                                                                                                                                                        |
| X <sub>1</sub> - (7)  |                                                                                                                                                                                        |
| X <sub>1</sub> - (8)  |                                                                                                                                                                                        |
| X <sub>1</sub> - (9)  |                                                                                                                                                                                        |
| X <sub>1</sub> - (10) |                                                                                                                                                                                        |
| X <sub>1</sub> - (11) |                                                                                                                                                                                        |
| X <sub>1</sub> - (12) |                                                                                                                                                                                        |
| X <sub>1</sub> - (13) |                                                                                                                                                                                        |
| X <sub>1</sub> - (14) |                                                                                                                                                                                        |
| X <sub>1</sub> - (15) |                                                                                                                                                                                        |
| X <sub>1</sub> - (16) |                                                                                                                                                                                        |
| X <sub>1</sub> - (17) |                                                                                                                                                                                        |
| X <sub>1</sub> - (18) |                                                                                                                                                                                        |
| X <sub>1</sub> - (19) |                                                                                                                                                                                        |
| X <sub>1</sub> - (20) |                                                                                                                                                                                        |
| X <sub>1</sub> - (21) |                                                                                                                                                                                        |
| X <sub>1</sub> - (22) |                                                                                                                                                                                        |
| X <sub>1</sub> - (23) |                                                                                                                                                                                        |
| X <sub>1</sub> - (24) |                                                                                                                                                                                        |
| X <sub>1</sub> - (25) |                                                                                                                                                                                        |
| X <sub>1</sub> - (26) |                                                                                                                                                                                        |
| X <sub>1</sub> - (27) |                                                                                                                                                                                        |
| X <sub>1</sub> - (28) |                                                                                                                                                                                        |
| X <sub>1</sub> - (29) |                                                                                                                                                                                        |
| X <sub>1</sub> - (30) |                                                                                                                                                                                        |
| X <sub>1</sub> - (31) |                                                                                                                                                                                        |
| X <sub>1</sub> - (32) |                                                                                                                                                                                        |
| X <sub>1</sub> - (33) |                                                                                                                                                                                        |
| X <sub>1</sub> - (34) |                                                                                                                                                                                        |
| X <sub>1</sub> - (35) |                                                                                                                                                                                        |
| X <sub>1</sub> - (36) |                                                                                                                                                                                        |
| X <sub>1</sub> - (37) |                                                                                                                                                                                        |
| X <sub>1</sub> - (38) |                                                                                                                                                                                        |
| X <sub>1</sub> - (39) |                                                                                                                                                                                        |
| X <sub>1</sub> - (40) |                                                                                                                                                                                        |
| X <sub>1</sub> - (41) |                                                                                                                                                                                        |

-continued

|                       |  |
|-----------------------|--|
| X <sub>1</sub> - (19) |  |
| X <sub>1</sub> - (20) |  |
| X <sub>1</sub> - (21) |  |
| X <sub>1</sub> - (22) |  |
| X <sub>1</sub> - (23) |  |
| X <sub>1</sub> - (24) |  |
| X <sub>1</sub> - (25) |  |
| X <sub>1</sub> - (26) |  |
| X <sub>1</sub> - (27) |  |
| X <sub>1</sub> - (28) |  |
| X <sub>1</sub> - (29) |  |
| X <sub>1</sub> - (30) |  |
| X <sub>1</sub> - (31) |  |

-continued

|                       |  |
|-----------------------|--|
| X <sub>1</sub> - (32) |  |
|-----------------------|--|

10 Examples of compounds represented by Formula (I) consisting of the cation part (T) and the anion part (X<sub>1</sub>) are listed below.

|        |                                                                                     |
|--------|-------------------------------------------------------------------------------------|
| I - 1  | 2,3-Diphenyl-5-(4-octyloxyphenyl)-2H-tetrazolium 3,5,5-trimethylhexylsulfosuccinate |
| I - 2  | 2,3,5-Tri(p-carboxyethylphenyl)-2H-tetrazolium 2,2-diethylhexylsulfosuccinate       |
| I - 3  | 2,3-Diphenyl-2H-tetrazolium dodecylbenzenesulfonate                                 |
| I - 4  | 2,3-Diphenyl-5-ethyl-2H-tetrazolium 3,5-didodecylbenzene-1-sulfonate                |
| I - 5  | 5-Cyano-2,3-diphenyl-2H-tetrazolium diisopropyl-naphthalenesulfonate                |
| I - 6  | 5-Ethoxycarbonyl-2,3-di(3-nitrophenyl)-2H-tetrazolium 1-methyl-benztriazolsulfonate |
| I - 7  | 2,5-Diphenyl-3-(p-tolyl)-2H-tetrazolium 2-mercaptopbenzoxazolsulfonate              |
| I - 8  | 2,3,5-Triphenyltetrazolium 3,5,5-trimethylhexylsulfosuccinate                       |
| I - 9  | 2,5-Diphenyl-3-(p-methoxyphenyl)tetrazolium t-amylsulfosuccinate                    |
| I - 10 | 2,3,5-Triphenyltetrazolium 2-mercaptopbenzo-imidazolsulfonate                       |
| I - 11 | 3-(p-Hydroxyphenyl)-5-methyl-2-phenyl-2H-tetrazolium cyclohexylsulfosuccinate       |
| I - 12 | 2,3-Diphenyl-5-(p-diphenyl)-2H-tetrazolium isopropylbenzenesulfosuccinate           |
| I - 13 | 2,3-Diphenyl-5-n-hexyl-2H-tetrazolium indazol-sulfonate                             |
| I - 14 | 2,3-Diphenyl-5-(p-ethylphenyl)-tetrazolium 2-octylbenzothiazolsulfosuccinate        |
| I - 15 | 2-(p-Nitrophenyl)-3,5-diphenyltetrazolium 1,5-dipropenylnaphthalenesulfonate        |

40 The compound represented by Formula (I) of this invention can be prepared by combining optionally a halide (e.g., chloride or bromide) containing the cation part T and an alkali metal (e.g., sodium or potassium) salt containing the anion part X<sub>1</sub>.

45 The halide containing the cation part T of this invention can be readily prepared, for instance, by the method described in Chemical Review, vol. 55, page 335-483.

50 Representative examples of the preparations of the compounds represented by Formula (I) are set forth below. Hereinafter percentage is represented by means of volume to volume.

#### EXAMPLE OF PREPARATION 1

55 To 1 liter of aqueous solution of 5-cyano-2,3-diphenyl-2H-tetrazolium chloride (5%) was added 500 ml of aqueous solution of diisopropylnaphthalenesulfonic acid (10%), and the resulting precipitate was collected by filtration, washed and dried to yield a product corresponding to Formula I-5.

#### EXAMPLE OF PREPARATION 2

60 To 1 liter of aqueous solution of 2,5-diphenyl-3-(p-tolyl)-2H-tetrazolium chloride (5%) was added little by little at room temperature 200 ml of aqueous 2-mercaptopbenzoxazolsulfonic acid (0.5%), and the resulting precipitate was collected by filtration, washed and dried to yield a product corresponding to Formula I-7.

## EXAMPLE OF PREPARATION 3

To 1 liter of aqueous solution of 2,3,5-triphenyltetrazolium chloride (5%) was added little by little at room temperature 350 ml of aqueous 3,5,5-trimethylhexylsulfosuccinic acid (5%), and the resulting mixture was placed in a separatory funnel. To the mixture was added 500 ml of chloroform, and after stirring the chloroform phase (underlayer) was separated. Upon evaporation of the chloroform by heating, there was obtained a product corresponding to Formula I-8. Reextract with chloroform yielded 36 g. of an oily product.

## EXAMPLE OF PREPARATION 4

To 1 liter of aqueous solution of 2,3,5-triphenyltetrazolium chloride (5%) was added little by little 600 ml of aqueous solution of 2-mercaptopbenzimidazol-5-sulfonic acid (1%), and the resulting precipitate was collected by filtration, washed and dried to yield a product corresponding to Formula I-10. Yield: 9.8 g.

## EXAMPLE OF PREPARATION 5

To 1 liter of a solution of 2-(p-nitrophenyl)-3,5-diphenyltetrazolium chloride in a mixture of fluorinated alcohol and water (5%) was added little by little 350 ml of 1,5-dipropenyl naphthalenesulfonate solution (5%), and the resulting precipitate was collected by filtration, washed and dried to yield a product corresponding to Formula I-15. Yield: 29 g.

The compound of Formula (I) which can be prepared by the methods stated in the above examples using a tetrazolium halide containing the cation part T (TX) and an alkali metal salt such as an alkali metal chloride containing the anion part X<sub>1</sub> (X<sub>1</sub>A) may be incorporated into a hydrophilic colloid of a light-sensitive silver halide photographic material. Alternatively, the compound TX and the compound X<sub>1</sub>A, both being in the form of an aqueous solution of an appropriate concentration, a solution in a water-miscible organic solvent such as methyl alcohol or fluorinated alcohol, or a dispersion in a gelatin matrix of latex, can be incorporated into a hydrophilic colloid of a light-sensitive silver halide photographic material.

In Formula (II), T represents a group as described for Formula (I), and m is an integer of 1 to 3. X<sub>2</sub> represents an atomic group or a group having the formulae (II-a), (II-b), (II-c), (II-d), (II-e), (II-f), (II-g) and (II-h).



Formula (II-a)



Formula (II-b)



Formula (II-c)



Formula (II-d)

10

-continued



Formula (II-e)



Formula (II-f)

Formula (II-g)



Formula (II-h)



In the above formulae (II-a) through (II-h), X<sub>1</sub>, X<sub>2</sub>, X<sub>3</sub>, X<sub>4</sub>, X<sub>5</sub>, X<sub>6</sub>, X<sub>7</sub>, X<sub>8</sub>, X<sub>9</sub>, X<sub>10</sub>, X<sub>11</sub>, X<sub>12</sub>, X<sub>13</sub>, X<sub>14</sub>, X<sub>15</sub>, X<sub>16</sub>, X<sub>17</sub>, X<sub>18</sub>, X<sub>19</sub>, X<sub>20</sub>, X<sub>21</sub>, X<sub>22</sub>, X<sub>23</sub>, X<sub>24</sub>, X<sub>25</sub>, X<sub>26</sub>, X<sub>27</sub>, X<sub>28</sub> and X<sub>29</sub>, which may be the same or different, represent groups  $-(CH_2)_{n17}COO^\ominus[T^\oplus]$  or  $-(CH_2)_{n17}COOH$  in which n<sub>17</sub> is an integer of 1 to 4. R in the formulae (II-b) and (II-h) represents alkyl such as methyl, ethyl or butyl, hydroxy, alkoxy,  $-NH_2$ ,  $-(CH_2)_{n17}COO^{63}[T^\oplus]$ ,  $-(CH_2)_{n17}COOH$ ,  $-PO_3H^\ominus[T^{61}]PO_3H_2$  in which T<sup>⊕</sup> has the same meaning as defined for Formula I.

20 30 In Formula (II-d), Z represents a group of atoms necessary to form a five- or six-membered ring, and the ring preferably consists of carbon, nitrogen, oxygen and/or sulfur atoms and more preferably is a five- or six-membered ring consisting of carbon atoms such as a cyclohexane or cyclopentane ring.

In the above-illustrated formulae n<sub>7</sub>, n<sub>8</sub>, n<sub>9</sub> and n<sub>11</sub>, which may be the same or different, are integers of 1 to 10.

40 45 In the formula (II-a) through (II-h), M represents a metal atom such as iron, cobalt, nickel, copper, manganese, lead, chromium, titanium, cerium, samarium, europium or ytterbium, and M preferably is such a metal atom as divalent copper, trivalent iron, cobalt, nickel, samarium, europium, chromium or ytterbium, or tetravalent titanium, cerium or lead, especially preferable are trivalent iron, cobalt and nickel.

50 55 A metal atom of the metal-chelate compound represented by Formula (II) is supposed to enhance the storage stability of the light-sensitive silver halide photographic material on the ground that other molecules (T and X<sub>2</sub> of the present invention) are connected to the metal by the coordination bond through the atomic bonding orbital of the metal in the form of octahedral, tetrahedral, planer or the like.

55 60 Examples of X<sub>2</sub><sup>m</sup> of Formula (II) representing the compound employed in this invention are listed below, but these examples are not intended to limit this invention.

## EXAMPLES

|                      |                                       |
|----------------------|---------------------------------------|
| (X <sub>2</sub> - 1) | Ethylenediaminetetraacetic acid       |
| (X <sub>2</sub> - 2) | Ethylenediaminetetraphosphoric acid   |
| (X <sub>2</sub> - 3) | 1,2-Propylenediaminetetraacetic acid  |
| (X <sub>2</sub> - 4) | Trimethylenediaminetetraacetic acid   |
| (X <sub>2</sub> - 5) | Tetramethylenediaminetetraacetic acid |
| (X <sub>2</sub> - 6) | Pentamethylenediaminetetraacetic acid |
| (X <sub>2</sub> - 7) | Hexamethylenediaminetetraacetic acid  |
| (X <sub>2</sub> - 8) | Octamethylenediaminetetraacetic acid  |

|                       |                                                                  |
|-----------------------|------------------------------------------------------------------|
| (X <sub>2</sub> - 9)  | 1,2-Cyclopentadiaminetetraacetic acid                            |
| (X <sub>2</sub> - 10) | Trans-cyclohexane-1,2-diaminetetraacetic acid                    |
| (X <sub>2</sub> - 11) | Cyclohexane-1,3-diaminetetraacetic acid                          |
| (X <sub>2</sub> - 12) | Cyclohexane-1,4-diaminetetraacetic acid                          |
| (X <sub>2</sub> - 13) | 1,3,5-Triaminocyclohexanetetraacetic acid                        |
| (X <sub>2</sub> - 14) | o-Phenylenediaminetetraacetic acid                               |
| (X <sub>2</sub> - 15) | 2-Hydroxytrimethylenediaminetetraacetic acid                     |
| (X <sub>2</sub> - 16) | Ethyl-ether-diaminetetraacetic acid                              |
| (X <sub>2</sub> - 17) | Ethyl-thioether-diaminetetraacetic acid                          |
| (X <sub>2</sub> - 18) | Diethylenetriaminepentaacetic acid                               |
| (X <sub>2</sub> - 19) | Glycol-ether-diaminetetraacetic acid                             |
| (X <sub>2</sub> - 20) | Thioglycol-thioether-diaminetetraacetic acid                     |
| (X <sub>2</sub> - 21) | N,N'-Dimethyltrimethylenetetraamine-N'',N'',N''-tetraacetic acid |
| (X <sub>2</sub> - 22) | Ethylenediamine-N,N'-diacetic acid-N,N'-dipropionic acid         |
| (X <sub>2</sub> - 23) | Trimethylenetetraaminehexaacid-nitrilotriacetic acid             |
| (X <sub>2</sub> - 24) | Carboxyethyliminodiacetic acid                                   |
| (X <sub>2</sub> - 25) | Carboxymethyliminodipropionic acid                               |
| (X <sub>2</sub> - 26) | Nitrilotripropionic acid                                         |

Examples of the compound represented by Formula (II) employed in this invention are listed below, but these examples are not intended to limit this invention.

### EXAMPLES

|         |                                                                                                 |
|---------|-------------------------------------------------------------------------------------------------|
| II - 1  | Cerium salt of diethylenetriaminepentaacetic acid-2,3,5-triphenyltetrazolium                    |
| II - 2  | Cobalt salt of glycol-ether-diaminetetraacetic acid-2,3-diphenyl-5-mercaptopotetrazolium        |
| II - 3  | Iron salt of ethylenediaminetetraacetic acid-2,3,5-triphenyltetrazolium                         |
| II - 4  | Iron salt of trans-cyclohexane-1,2-diaminetetraacetic acid-2,3,5-triphenyltetrazolium           |
| II - 5  | Cobalt salt of ethylenediaminetetraacetic acid-2-(tolyl)-3,5-diphenyltetrazolium                |
| II - 6  | Iron salt of ethylenediaminetetrapropionic acid-2,3-diphenyl-5-mercaptopotetrazolium            |
| II - 7  | Iron salt of ethyl-ether-diaminetetraacetic acid-2,3-carboxy-5-phenyltetrazolium                |
| II - 8  | Lead salt of pentamethylenediaminetetraacetic acid-2,3-hydroxy-5-phenyltetrazolium              |
| II - 9  | Copper salt of hexamethylenediaminetetraacetic acid-2,3,5-triphenyltetrazolium                  |
| II - 10 | Europium salt of ethylenediaminetetraacetic acid-2-(p-hydroxyphenyl)-3,5-diphenyltetrazolium    |
| II - 11 | Ytterbium salt of trimethylenediaminetetraacetic acid-2-(p-nitrophenyl)-3,5-diphenyltetrazolium |
| II - 12 | Ytterbium salt of ethylenediaminetetraacetic acid-2,3,5-triphenyltetrazolium                    |
| II - 13 | Cobalt salt of ethylenediaminetetraacetic acid-2,3-diphenyl-5-cyanotetrazolium                  |
| II - 14 | Samarium salt of ethylenediaminetetraacetic acid-2,3,5-triphenyltetrazolium                     |
| II - 15 | Nickel salt of ethylenediaminetetraacetic acid-2,3-diphenyl-5-(p-methylphenyl)tetrazolium       |
| II - 16 | Cerium salt of ethylenediaminetetraacetic acid-2,3,5-triphenyltetrazolium                       |
| II - 17 | Iron salt of 2-hydroxytrimethylenediaminetetraacetic acid-2,3,5-triphenyltetrazolium            |
| II - 18 | Iron salt of ethylenediaminetetraacetic acid-2,3,5-triphenyltetrazolium                         |
| II - 19 | Cobalt salt of ethylenediaminetetraacetic acid-2,3,5-triphenyltetrazolium                       |
| II - 20 | Iron salt of ethylenediaminetetraphosphoric acid-2,3,5-triphenyltetrazolium                     |

The compound represented by Formula (II) of this invention can be readily prepared, in the same manner for the preparation of the compound represented by Formula (I), by combining optionally a halide (e.g., chloride or bromide) containing the cation part T and

an alkali metal salt of the metal-chelate compound containing the anion part X<sub>2</sub>.

The compound of Formula (II) which can be prepared by using a tetrazolium halide TX containing the cation part T and an alkali metal salt of the metal-chelate compound X<sub>2</sub>K containing the anion part X<sub>2</sub> may be incorporated into a hydrophilic colloid of a light-sensitive silver halide photographic material, wherein X and T represent a halogen atom and an alkali metal, respectively. Alternatively, the compound TX and the compound X<sub>2</sub>K, each in the form in a solution of an appropriate solvent or a dispersion in a latex of a gelatin matrix, can be incorporated into a hydrophilic colloid of a light-sensitive silver halide photographic material, whereby the compound of Formula (II) is prepared.

The light-sensitive silver halide photographic material of this invention comprises a support, and on the support a hydrophilic colloidal layer comprising at least one silver halide emulsion layer is coated. The silver halide emulsion layer can be coated on a support directly, or firstly a hydrophilic colloidal layer comprising no silver halide emulsion layer is coated on a support, secondly a silver halide emulsion layer is coated thereon, and lastly a hydrophilic colloidal layer is coated thereon for protection. The silver halide emulsion layer can be divided to become two or more layers, and in this case an intermediate layer can be placed between the multiple silver halide emulsion layers or between the silver halide emulsion layers and the protective layer. The layer in which the compound of this invention is incorporated is a hydrophilic colloidal layer, and preferably is either or both of the silver halide emulsion layer and/or a hydrophilic colloidal layer adjacent to said silver halide emulsion layer.

The compounds represented by Formula (I) and Formula (II) are incorporated in the silver halide emulsion layer respectively in an amount ranging from  $10^{-4}$  to  $10^{-1}$  mol/mol of silver, preferably from  $10^{-3}$  to  $10^{-2}$  mol/mol of silver, and more preferably from  $5 \times 10^{-3}$  to  $5 \times 10^{-2}$  mol/mol of silver. The ratio of the compound of Formula (I) against the compound of Formula (II) is preferably from  $10^{-3}$  to  $10^3$  and more preferably from  $10^{-1}$  to 10. The compound of Formula (I) and the compound of Formula (II) can be incorporated in the silver halide emulsion in a manner usually adopted for incorporation of additives into a silver halide emulsion. For instance, if the compound is soluble in water, it can be incorporated in the form of an aqueous solution of an appropriate concentration. If the compound is not or sparingly soluble in water, it can be incorporated in the form of a solution in a water-miscible organic solvent such as an alcohol, an ether, a glycol, an acetone, an ester, an amine or the like. Otherwise employed, for instance, is a known method for incorporating a water-insoluble coupler into the emulsion in the form a dispersion.

The compound of this invention can be incorporated in a single silver halide emulsion layer or in multiple silver halide emulsion layers. The compound of Formula (I) and the compound of Formula (II) can be together incorporated in a single layer or separately incorporated in multiple layers. If the compound of Formula (I) and/or the compound of Formula (II) are incorporated in a light-insensitive hydrophilic colloidal layer, said layer can be selected optionally from an intermediate layer, a protecting layer, a backing layer, etc.

A preferable embodiment of a photographic material of the present invention contains a hydrophilic colloidal layer containing a silver halide emulsion and a hydrophilic colloidal layer containing no silver halide emulsion coated on a support at this order and one layer is adjacent to the other. Further preferably both layers contain the compounds of the Formulae (I) and (II), and a concentration of total amount of the said compound to a hydrophilic colloid of the hydrophilic colloidal layer containing no silver halide emulsion is from 1.2 to 10 times greater than the concentration of the hydrophilic colloidal layer containing a silver halide emulsion.

Examples of the silver halide employed in this invention include silver chloride, silver chlorobromide, silver iodochlorobromide, silver bromide and silver iodobromide. If silver chlorobromide or silver iodochlorobromide is employed, silver bromide contained in it is preferably up to 50 mol %. If silver iodobromide or silver iodochlorobromide is employed, silver iodide contained in it is preferably up to 10 mole %.

The silver halide used for practising the present invention can be prepared in any methods known to a person skill in the art. The silver halide can be advantageously applied such methods as the conversion method disclosed in U.S. Pat. No. 2,592,250 and the shelling method disclosed in Japanese Patent Provisional Publication 50(1978)-56,226 so as to enhance the developing capacity at a higher exposed part.

For the purpose of accomplishing higher contrast, a narrower range of the silver halide grain size distribution is preferred and, particularly, sizes of 80% of the whole number of the grains are preferably within the range of  $\pm 40\%$  deviation from the average grain size with respect to the weight and number of the silver halide grains. For this reason, the preparation of the silver halide is preferably carried out by the pAg regulating simultaneous mixing method in which the reaction between a water-soluble silver salt and a water-soluble halide is done in a liquid phase maintaining the pAg constant or by the functionally adding simultaneous mixing method in which a water-soluble silver salt and a water-soluble halide are added in amounts varying proportionally to the surface area of the silver halide under crystal growing. The average grain size of the obtained silver halide preferably is smaller from the viewpoints of the development progress and halftone formation, but preferably is larger from the viewpoint of the sensitivity. The average grain size satisfying these requests is within  $0.15\mu$  to  $0.8\mu$ .

In the process for preparing the photographic material involving the compounds of this invention, two or more kinds of silver halides can be employed after mixing, or each of these silver halides can be successively overlaid in the form of a separated layer.

When the silver halide grains are being formed or being physically ripened, a cadmium salt, a zinc salt, a lead salt, a thallium salt, an iridium salt, an iridium complex salt, a rhodium salt, a rhodium complex salt, an iron salt, an iron complex salt, etc. can be together present in the phase.

The silver halide emulsion employed in this invention can be sensitized by the use of a variety of chemical sensitizers.

The silver halide emulsion used in this invention is 65 optically sensitized by the use of one or more sensitizing dyes so as to impart the emulsion the sensitivity in the desired wavelength area.

The hydrophilic colloid which forms the hydrophilic colloidal layer is generally made of gelatin. Said hydrophilic colloid can be applied to such layers containing no silver halide as antihalation layer, protective layer, intermediate layer, underlayer, filter layer, backing layer, etc. The preferred hydrophilic colloids are gelatin and/or the gelatin derivatives.

The light-sensitive silver halide photographic material of this invention can be prepared by coating the aforementioned layers on an appropriate photographic support. Examples of the support include baryta paper, polyethylene-coated paper, synthetic polypropylene paper, glass plate, cellulose acetate film, cellulose nitrate film, polyester film such as polyethylene terephthalate film, etc. The support is optionally selected depending on the purpose for which the light-sensitive photographic material is employed.

As stated above, the light-sensitive silver halide photographic material of this invention comprises at least 20 one hydrophilic colloidal layer containing silver halide coated on a support. Preferably, the light-sensitive silver halide photographic material of this invention is coated with a protective layer generally made of gelatin having an appropriate film thickness, for instance, 25  $0.1\mu$ - $10\mu$ , preferably  $0.8\mu$ - $2\mu$ .

Previously known lith-type light-sensitive silver halide photographic materials generally contain protective layers. However, the protective layer which may be employed in this invention serves for imparting a very 30 important function being different from the functions usually known.

In a general sense, the protective layer is provided for protecting the silver halide emulsion layer from undesired damages, for example, damages received in the 35 cutting, rolling and packing stages in the process for the preparation of light-sensitive silver halide photographic materials or damages received by contacts of the photographic material with other materials in the course of taking picture or processing. The protective layer 40 optionally applied to the invention serves an important role for the processing stability as well as the role stated above. The reason why the protective layer can effectively function for stabilizing the quality of images and development is not known. It is assumed that the protective layer can effectively control the penetrating rate 45 of such a developing agent as hydroquinone, Metol (R)(p-methylaminophenol sulfate) or Phenidone (R)(1-phenyl-3-pyrazolidone) from the processing solution to the light-sensitive silver halide photographic 50 material, the diffusion property of the compounds of Formula (I) and Formula (II) in the photographic material, or the diffusion property of said compounds from the photographic material to the processing solution.

An image can be obtained by exposing and then 55 processing the photographic material of the present invention. The image obtained according to the process using the photographic material of this invention is a silver image with high contrast. Therefore, the present invention can be applied in the art that requires the high 60 contrast black-and-white recording, and preferably is employed as light-sensitive materials for the printing use, microphotography, etc. The present invention provides excellent characteristics in the formation of the lith-type photographic image as compared with the conventional art.

The developer employed for the process involving the material of this invention is, not necessarily, the so-called lith-type developer, and even in the presence

of a sulfite ion of a high concentration the high-contrast silver image can be obtained. This process does not require, but may employ, conventional hydroquinone, alkali, alkali metal bromide and a sulfite ion of a low concentration, as well as such a preserving agent as formaldehyde-sodium bisulfite or a carbonyl bisulfite-amine condensation which are conventionally employed in the so-called lith-type developing agent. The developer containing the developing agent employed for the present invention is not only the so-called lith-type developer but also the so-called MQ or PQ developer. Said MQ or PQ developer is advantageously used in the present process due to excellency in the preparation and preservation of the solution.

The developing agents described in C.E.K. Mees, T. H. James: The Theory of the Photographic Process, 3rd Ed., pages 278-311, and in Journal of the American Chemical Society, 73, 3100 (1951) are effectively employed for the present process.

The developing agent can be applied singly or in combination of two or more kinds. The latter is preferred. Examples of the preferred developing agent include a hydroquinone type, a p-aminophenol type, a 3-pyrazolidone type and a p-phenylenediamine type. The developing solution employed in this process can contain sodium sulfite, potassium sulfite, ammonium sulfite, or other sulfites as the preserving agent, not disturbing the effect of the present invention. This is one of the characteristics of this invention. The sulfite is preferably contained in a developer in an amount of  $1 \times 10^{-1.1}$  mol/l. Such a preserving agent as hydroxylamine, ethanolamine, alkanolamine sulfite adduct or hydrazide can be also contained. Also optionally added are the pH regulator such as a caustic alkali, an alkali carbonate being preferably added to the developer in an amount of  $1 \times 10^{-1.2}$  mol/l, or an amine, such pH regulators being capable of functioning as buffers, an inorganic development retarder such as potassium bromide, an organic development retarder such as a triazol, tetrazol, benzimidazole, benztriazole, benzthiazole, benzoxazole, and indazole, a metal ion capturer (sequestering agent) such as ethylenediaminetetraacetate, a developing accelerator such as methanol, ethanol, benzyl alcohol or polyalkylene oxide, a surfactant such as sodium alkylarylsulfonate, a hardening agent such as glutaraldehyde, formalin or glyoxal, and an ion strength regulator such as sodium sulfate.

The light-sensitive silver halide photographic material of this invention can be processed under different conditions. The temperature of the developer in the course of the processing generally ranges from 15° to 60° C., preferably is around 30° C. The developing time is generally up to 10 minutes, and the period of up to 5 minutes is preferred to achieve a satisfactory result. The developer preferably has pH 8 to 12, more preferably pH 9 to 11. Optionally employed and optionally omitted are other stages than the developing such as the washing with water, stopping, stabilizing, fixing, pre-hardening and neutralizing.

The one preferred embodiment of this invention showed the storage stability of more than twenty times as long as that of the conventional lith-type developer, both having been determined in the plate processing. The conventional special developer that contains an extremely reduced sulfite concentration, that is, the lith-type developer, and that is employed to improve the halftone property of the lith-type light-sensitive silver halide photographic material so deteriorates

within a few hours that it cannot be practically used. In contrast, a preferred embodiment of the developer of this invention can be still used practically after one month or more, maintaining the halftone property almost similar to that yielded by the use of a fresh developer. To the developer used for this invention can be added such additives as ones generally added to the conventional high-contrast developer, for instance, a high contrasting agent and an agent reducing a density at low density part.

The light-sensitive silver halide photographic material composed as stated hereinbefore has high contrast and excellent storage stability as described above. Moreover, it can improve other characteristics in the processing: that is, (1) reduction of unevenness of development due to uniform stirring of the developer during the processing, (2) making the developing speed moderate to eliminate a steep growing of fog in the latter period of the development and (3) improving the reduction of a silver image of the sample after the processing.

This invention will be further illustrated by the following examples including the reference examples, but these examples are not to be intended to limit this invention. Therefore, this invention can be embodied in different ways within the claims.

#### EXAMPLE 1

A gelatin emulsion of silver chlorobromide (silver chloride: 90 mole %, silver bromide: 10 mole %, average grain size:  $0.3\mu$ ) 90% of which grain total number had the grain size of 0.7 to 1.3 times as much as the average grain size was chemically sensitized with a sulfur sensitizing agent and a gold sensitizing agent. The obtained emulsion was divided into several portions, and to each were added the compounds of this invention as shown in Table 1, a coating aid and a hardening agent.

The emulsion was then coated on a support made of polyethylene terephthalate in the ratios of 50 mg of silver and 35 mg of gelatin per 100 cm<sup>2</sup> of the area of the support. On the resulting silver halide emulsion layer was coated a protective gelatin layer (15 mg/100 cm<sup>2</sup>), and the obtained sample was further treated as follows.

For comparison of the photographic characteristics, the sample thus obtained was wedge-exposed through the tungsten light contact screen (150 L chain-dot type for the preparation of negative) and treated in the manner described below.

The storage stability of the sample was examined as follows: The coated and dried sample was kept for 24 hours in a room at a relative humidity (RH) of 50% and a temperature of 23° C. In the same room, the sample was then inserted into an air-tight envelop for the light-sensitive material, kept for one day or ten days in a preserving vessel maintained at 65° C., and taken out for exposure and development. Another sample was prepared by keeping in a room at RH 50% and 23° C. The other sample was, in contrast, exposed and developed immediately after the coating and drying. After the processing, these samples were examined on their photographic characteristics.

The quality of halftone was judged by examining microscopically the dot-image. The balckened concentration 50% part, namely, the almost central part between the shadow part and the highlight part, was examined, and the marks 7 and 1 were given to the best and the worst, respectively. Between the best and the

worst, seven ranks were allotted. The relative sensitivity was calculated based on the quantity of light required for giving the blackened concentration 50%. The results are set out in Table 1. The examination as to the storage stability and the quality of halftone are applied to other Examples.

Processing details (30 min.)

Development (1 min.) - Fixing (1 min.) - Washing with water (1 min.) - Drying (40 sec.)

Developer

|                                        |       |
|----------------------------------------|-------|
| Methol ® (p-methylaminophenol sulfate) | 3.5 g |
| Anhydrous sodium sulfite               | 50 g  |
| Hydroquinone                           | 10 g  |
| Sodium carbonate . monohydrate         | 50 g  |
| Potassium bromide                      | 3 g   |
| Sodium ethylenediaminetetraacetate     | 0.5 g |
| 5-Nitroindazole                        | 60 mg |

Water was added to make the volume to one liter and this was then adjusted to pH 10.0.

Fixing solution

|                                    |       |
|------------------------------------|-------|
| Ammonium thiosulfate . 10 hydrates | 150 g |
| Anhydrous sodium sulfite           | 10 g  |
| Sodium acetate . 3 hydrates        | 15 g  |
| Glacial acetic acid                | 17 g  |

Water was added to make the volume to one liter and this was then adjusted to pH 4.20.

(I) has satisfactory photographic characteristics not only when processed just after the coating but also when processed after standing.

**EXAMPLE 2**

A gelatin emulsion of silver bromide (average grain size:  $0.35\mu$ ) 90% of which grain total number had the grain sizes ranging from  $0.25\mu$  to  $0.45\mu$  was chemically sensitized with a sulfur sensitizing agent and a gold sensitizing agent. The obtained emulsion was divided into several portions, and to each were added the compounds of this invention as shown in Table 2, a coating aid, a stabilizer, an antifoggant, and a hardening agent.

The emulsion was then coated on a support made of polyethylene terephthalate in the ratios of 48 mg. of silver and 38 mg. of gelatin per  $100\text{ cm}^2$  of the area of the support. On the resulting silver halide emulsion layer was coated a protective gelatin layer (15 mg/ $100\text{ cm}^2$ ), and the obtained sample was preserved, exposed and processed in the manner as employed in Example 1, except that the developer of the following formulation was used instead of the one stated in Example 1. The results are set out in Table 2.

Developer

TABLE I

| Sam-<br>ple | Compound of<br>Formula (I)<br>(mol/mol Ag) | Compound of<br>Formula (II)<br>(mol/mol Ag) | Preserving Conditions        |                      |                          |      |                  |     |                          |     |                                        |      |                          |     |      |     |
|-------------|--------------------------------------------|---------------------------------------------|------------------------------|----------------------|--------------------------|------|------------------|-----|--------------------------|-----|----------------------------------------|------|--------------------------|-----|------|-----|
|             |                                            |                                             | 23° C., RH 50%               |                      |                          |      |                  |     |                          |     |                                        |      |                          |     |      |     |
|             |                                            |                                             | Immediately<br>after coating |                      |                          |      | After 6 months   |     |                          |     | Enveloped sample (preserved at 65° C.) |      |                          |     |      |     |
|             |                                            |                                             | Sensi-<br>tivity             | Fog                  | Half-<br>tone<br>quality |      | Sensi-<br>tivity | Fog | Half-<br>tone<br>quality |     | Sensi-<br>tivity                       | Fog  | Half-<br>tone<br>quality |     |      |     |
| 1           | I - 10                                     | $1 \times 10^{-3}$                          |                              |                      | 100                      | 0.04 | 7                | 250 | 0.50                     | 3   | 260                                    | 0.90 | 3                        | 300 | 1.0  | 1   |
| 2           | I - 2                                      | $2 \times 10^{-3}$                          | II - 8                       | $2.3 \times 10^{-4}$ | 100                      | 0.04 | 7                | 100 | 0.04                     | 7   | 100                                    | 0.04 | 7                        | 103 | 0.04 | 6   |
| 3           | I - 2                                      | $1 \times 10^{-3}$                          | II - 3                       | $4 \times 10^{-4}$   | 102                      | 0.04 | 7                | 100 | 0.04                     | 7   | 100                                    | 0.04 | 7                        | 100 | 0.03 | 6   |
|             | I - 5                                      | $1 \times 10^{-5}$                          |                              |                      |                          |      |                  |     |                          |     |                                        |      |                          |     |      |     |
| 4           | I - 4                                      | $1.3 \times 10^{-3}$                        | II - 6                       | $3 \times 10^{-5}$   | 101                      | 0.04 | 6                | 98  | 0.04                     | 6   | 98                                     | 0.04 | 6                        | 110 | 0.04 | 6   |
| 5           | I - 3                                      | $2 \times 10^{-3}$                          | II - 5                       | $1.5 \times 10^{-3}$ | 100                      | 0.04 | 7                | 102 | 0.04                     | 6.5 | 102                                    | 0.04 | 6.5                      | 103 | 0.04 | 6.5 |
| 6           | I - 6                                      | $3 \times 10^{-4}$                          | II - 7                       | $3 \times 10^{-3}$   | 101                      | 0.04 | 6.5              | 102 | 0.04                     | 6.3 | 102                                    | 0.04 | 6.5                      | 95  | 0.04 | 6.3 |
| 7           | I - 7                                      | $2 \times 10^{-3}$                          | II - 9                       | $2.3 \times 10^{-3}$ | 100                      | 0.04 | 6                | 100 | 0.04                     | 6   | 100                                    | 0.04 | 6                        | 95  | 0.04 | 6   |
| 8           | I - 10                                     | $2.3 \times 10^{-3}$                        | II - 4                       | $4 \times 10^{-4}$   | 100                      | 0.07 | 6                | 97  | 0.03                     | 6   | 97                                     | 0.04 | 6                        | 100 | 0.04 | 6   |
| 9           | I - 12                                     | $5 \times 10^{-3}$                          | II - 13                      | $1.5 \times 10^{-3}$ | 100                      | 0.04 | 7                | 105 | 0.04                     | 7   | 103                                    | 0.04 | 7                        | 103 | 0.04 | 6.5 |
| 10          | I - 15                                     | $1.5 \times 10^{-3}$                        | II - 15                      | $2.0 \times 10^{-3}$ | 102                      | 0.04 | 6.5              | 103 | 0.03                     | 6.5 | 103                                    | 0.04 | 6.5                      | 105 | 0.04 | 6.5 |

As seen from the results set out in Table 1, the sample containing only the compound of Formula (I) has higher halftone quality and shows less fog when it is processed just after the coating. After allowing to stand for six months at 25° C. and 50%, RH, or keeping for 50 one or ten days at 65° C. in a sealed envelop, the halftone quality lowers, the fog increases and the sensitivity varies, all these changes being apparent.

In contrast, the sample containing the compound of Formula (II) together with the compound of Formula

|                                       |        |
|---------------------------------------|--------|
| Phenidone ® (1-phenyl-3-pyrazolidone) | 3 g.   |
| Anhydrous sodium sulfite              | 60 g.  |
| Hydroquinone                          | 10 g.  |
| Sodium carbonate . monohydrate        | 50 g.  |
| Potassium bromide                     | 2.5 g. |
| Sodium ethylenediaminetetraacetate    | 1.0 g. |
| 5-Nitrobenzimidazole                  | 5 g.   |

Water was added to make the volume to one liter and this was then adjusted to pH 10.8.

TABLE 2

| Sam-<br>ple | Compound of<br>Formula (I)<br>(mol/mol Ag) | Compound of<br>Formula (II)<br>(mol/mol Ag) | Preserving Conditions        |                      |                          |      |                  |     |                          |   |                                        |      |                          |     |      |     |
|-------------|--------------------------------------------|---------------------------------------------|------------------------------|----------------------|--------------------------|------|------------------|-----|--------------------------|---|----------------------------------------|------|--------------------------|-----|------|-----|
|             |                                            |                                             | 23° C., RH 50%               |                      |                          |      |                  |     |                          |   |                                        |      |                          |     |      |     |
|             |                                            |                                             | Immediately<br>after coating |                      |                          |      | After 6 months   |     |                          |   | Enveloped sample (preserved at 65° C.) |      |                          |     |      |     |
|             |                                            |                                             | Sensi-<br>tivity             | Fog                  | Half-<br>tone<br>quality |      | Sensi-<br>tivity | Fog | Half-<br>tone<br>quality |   | Sensi-<br>tivity                       | Fog  | Half-<br>tone<br>quality |     |      |     |
| 1           | I - 3                                      | $2 \times 10^{-3}$                          |                              |                      | 100                      | 0.04 | 7                | 250 | 0.50                     | 3 | 260                                    | 0.90 | 3                        | 300 | 1.0  | 1   |
| 2           | I - 5                                      | $2 \times 10^{-2}$                          | II - 1                       | $2 \times 10^{-3}$   | 100                      | 0.04 | 7                | 100 | 0.04                     | 7 | 100                                    | 0.04 | 6                        | 98  | 0.05 | 6   |
|             |                                            |                                             | II - 2                       | $0.5 \times 10^{-3}$ |                          |      |                  |     |                          |   |                                        |      |                          |     |      |     |
| 3           | I - 6                                      | $3 \times 10^{-3}$                          | II - 3                       | $3 \times 10^{-3}$   | 100                      | 0.04 | 7                | 100 | 0.04                     | 7 | 100                                    | 0.04 | 6                        | 97  | 0.04 | 6   |
| 4           | I - 7                                      | $3 \times 10^{-3}$                          | II - 2                       | $2.5 \times 10^{-3}$ | 100                      | 0.04 | 6                | 99  | 0.03                     | 6 | 98                                     | 0.04 | 5.9                      | 98  | 0.05 | 5.8 |
| 5           | I - 10                                     | $2.5 \times 10^{-3}$                        | II - 5                       | $2 \times 10^{-3}$   | 101                      | 0.04 | 6                | 100 | 0.03                     | 6 | 97                                     | 0.04 | 6                        | 97  | 0.04 | 6   |

TABLE 2-continued

| Sam-<br>ple | Compound of<br>Formula (I)<br>(mol/mol Ag) | Compound of<br>Formula (II)<br>(mol/mol Ag) | Preserving Conditions        |                      |                          |                  |     |                          |                                        |     |                          |                  |     |                          |      |     |
|-------------|--------------------------------------------|---------------------------------------------|------------------------------|----------------------|--------------------------|------------------|-----|--------------------------|----------------------------------------|-----|--------------------------|------------------|-----|--------------------------|------|-----|
|             |                                            |                                             | 23° C., RH 50%               |                      |                          |                  |     |                          | Enveloped sample (preserved at 65° C.) |     |                          |                  |     |                          |      |     |
|             |                                            |                                             | Immediately<br>after coating |                      |                          | After 6 months   |     |                          | One day                                |     |                          | Ten days         |     |                          |      |     |
|             |                                            |                                             | Sensi-<br>tivity             | Fog                  | Half-<br>tone<br>quality | Sensi-<br>tivity | Fog | Half-<br>tone<br>quality | Sensi-<br>tivity                       | Fog | Half-<br>tone<br>quality | Sensi-<br>tivity | Fog | Half-<br>tone<br>quality |      |     |
| 6           | I - 15                                     | $2.5 \times 10^{-3}$                        | II - 6                       | $2 \times 10^{-3}$   | 103                      | 0.04             | 6.5 | 105                      | 0.04                                   | 6.3 | 100                      | 0.04             | 6.3 | 99                       | 0.04 | 6.0 |
| 7           | I - 13                                     | $3 \times 10^{-4}$                          | II - 7                       | $2 \times 10^{-3}$   | 102                      | 0.04             | 7   | 100                      | 0.05                                   | 7   | 98                       | 0.04             | 6.8 | 95                       | 0.03 | 6.5 |
| 8           | I - 11                                     | $3 \times 10^{-4}$                          | II - 8                       | $3.5 \times 10^{-3}$ | 98                       | 0.04             | 7   | 100                      | 0.04                                   | 7   | 98                       | 0.04             | 7   | 98                       | 0.04 | 6   |
| 9           | I - 9                                      | $2 \times 10^{-3}$                          | II - 10                      | $2 \times 10^{-3}$   | 100                      | 0.04             | 6.5 | 103                      | 0.05                                   | 6.5 | 99                       | 0.04             | 6.5 | 99                       | 0.04 | 6   |
| 10          | I - 1                                      | $2 \times 10^{-3}$                          | II - 13                      | $2 \times 10^{-3}$   | 102                      | 0.04             | 7   | 102                      | 0.05                                   | 7   | 100                      | 0.04             | 7   | 100                      | 0.04 | 7   |

As seen from the results set out in Table 1, the sample containing only the compound of Formula (I) has higher halftone quality and shows less fog when it is processed just after the coating. After allowing to stand for six months at 25° C. and 50% RH, or keeping for one or ten days at 65° C. in a sealed envelop, the halftone quality lowers, the fog increases and the sensitivity varies, all these changes being apparent.

In contrast, the sample containing the compound of

15  
16  
17  
18  
19  
20  
21  
22  
23  
24  
25  
26  
27  
28  
29  
30  
31  
32  
33  
34  
35  
36  
37  
38  
39  
40  
41  
42  
43  
44  
45  
46  
47  
48  
49  
50  
51  
52  
53  
54  
55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
339  
340  
341  
342  
343  
344  
345  
346  
347  
348  
349  
349  
350  
351  
352  
353  
354  
355  
356  
357  
358  
359  
359  
360  
361  
362  
363  
364  
365  
366  
367  
368  
369  
369  
370  
371  
372  
373  
374  
375  
376  
377  
378  
379  
379  
380  
381  
382  
383  
384  
385  
386  
387  
388  
389  
389  
390  
391  
392  
393  
394  
395  
396  
397  
398  
399  
399  
400  
401  
402  
403  
404  
405  
406  
407  
408  
409  
409  
410  
411  
412  
413  
414  
415  
416  
417  
418  
419  
419  
420  
421  
422  
423  
424  
425  
426  
427  
428  
429  
429  
430  
431  
432  
433  
434  
435  
436  
437  
438  
439  
439  
440  
441  
442  
443  
444  
445  
446  
447  
448  
449  
449  
450  
451  
452  
453  
454  
455  
456  
457  
458  
459  
459  
460  
461  
462  
463  
464  
465  
466  
467  
468  
469  
469  
470  
471  
472  
473  
474  
475  
476  
477  
478  
479  
479  
480  
481  
482  
483  
484  
485  
486  
487  
488  
489  
489  
490  
491  
492  
493  
494  
495  
496  
497  
498  
499  
499  
500  
501  
502  
503  
504  
505  
506  
507  
508  
509  
509  
510  
511  
512  
513  
514  
515  
516  
517  
518  
519  
519  
520  
521  
522  
523  
524  
525  
526  
527  
528  
529  
529  
530  
531  
532  
533  
534  
535  
536  
537  
538  
539  
539  
540  
541  
542  
543  
544  
545  
546  
547  
548  
549  
549  
550  
551  
552  
553  
554  
555  
556  
557  
558  
559  
559  
560  
561  
562  
563  
564  
565  
566  
567  
568  
569  
569  
570  
571  
572  
573  
574  
575  
576  
577  
578  
579  
579  
580  
581  
582  
583  
584  
585  
586  
587  
588  
589  
589  
590  
591  
592  
593  
594  
595  
596  
597  
598  
599  
599  
600  
601  
602  
603  
604  
605  
606  
607  
608  
609  
609  
610  
611  
612  
613  
614  
615  
616  
617  
618  
619  
619  
620  
621  
622  
623  
624  
625  
626  
627  
628  
629  
629  
630  
631  
632  
633  
634  
635  
636  
637  
638  
639  
639  
640  
641  
642  
643  
644  
645  
646  
647  
648  
649  
649  
650  
651  
652  
653  
654  
655  
656  
657  
658  
659  
659  
660  
661  
662  
663  
664  
665  
666  
667  
668  
669  
669  
670  
671  
672  
673  
674  
675  
676  
677  
678  
679  
679  
680  
681  
682  
683  
684  
685  
686  
687  
688  
689  
689  
690  
691  
692  
693  
694  
695  
696  
697  
697  
698  
699  
699  
700  
701  
702  
703  
704  
705  
706  
707  
708  
709  
709  
710  
711  
712  
713  
714  
715  
716  
717  
718  
719  
719  
720  
721  
722  
723  
724  
725  
726  
727  
728  
729  
729  
730  
731  
732  
733  
734  
735  
736  
737  
738  
739  
739  
740  
741  
742  
743  
744  
745  
746  
747  
748  
749  
749  
750  
751  
752  
753  
754  
755  
756  
757  
758  
759  
759  
760  
761  
762  
763  
764  
765  
766  
767  
768  
769  
769  
770  
771  
772  
773  
774  
775  
776  
777  
778  
778  
779  
779  
780  
781  
782  
783  
784  
785  
786  
787  
788  
789  
789  
790  
791  
792  
793  
794  
795  
796  
797  
797  
798  
799  
799  
800  
801  
802  
803  
804  
805  
806  
807  
808  
809  
809  
810  
811  
812  
813  
814  
815  
816  
817  
818  
819  
819  
820  
821  
822  
823  
824  
825  
826  
827  
828  
829  
829  
830  
831  
832  
833  
834  
835  
836  
837  
838  
839  
839  
840  
841  
842  
843  
844  
845  
846  
847  
848  
849  
849  
850  
851  
852  
853  
854  
855  
856  
857  
858  
859  
859  
860  
861  
862  
863  
864  
865  
866  
867  
868  
869  
869  
870  
871  
872  
873  
874  
875  
876  
877  
878  
878  
879  
879  
880  
881  
882  
883  
884  
885  
886  
887  
888  
889  
889  
890  
891  
892  
893  
894  
895  
896  
897  
897  
898  
899  
899  
900  
901  
902  
903  
904  
905  
906  
907  
908  
909  
909  
910  
911  
912  
913  
914  
915  
916  
917  
918  
919  
919  
920  
921  
922  
923  
924  
925  
926  
927  
928  
929  
929  
930  
931  
932  
933  
934  
935  
936  
937  
938  
939  
939  
940  
941  
942  
943  
944  
945  
946  
947  
948  
949  
949  
950  
951  
952  
953  
954  
955  
956  
957  
958  
959  
959  
960  
961  
962  
963  
964  
965  
966  
967  
968  
969  
969  
970  
971  
972  
973  
974  
975  
976  
977  
978  
978  
979  
979  
980  
981  
982  
983  
984  
985  
986  
987  
988  
989  
989  
990  
991  
992  
993  
994  
995  
996  
997  
997  
998  
999  
999  
1000  
1001  
1002  
1003  
1004  
1005  
1006  
1007  
1008  
1009  
1009  
1010  
1011  
1012  
1013  
1014  
1015  
1016  
1017  
1018  
1019  
1019  
1020  
1021  
1022  
1023  
1024  
1025  
1026  
1027  
1028  
1029  
1029  
1030  
1031  
1032  
1033  
1034  
1035  
1036  
1037  
1038  
1039  
1039  
1040  
1041  
1042  
1043  
1044  
1045  
1046  
1047  
1048  
1049  
1049  
1050  
1051  
1052  
1053  
1054  
1055  
1056  
1057  
1058  
1059  
1059  
1060  
1061  
1062  
1063  
1064  
1065  
1066  
1067  
1068  
1069  
1069  
1070  
1071  
1072  
1073  
1074  
1075  
1076  
1077  
1078  
1078  
1079  
1079  
1080  
1081  
1082  
1083  
1084  
1085  
1086  
1087  
1088  
1089  
1089  
1090  
1091  
1092  
1093  
1094  
1095  
1096  
1097  
1097  
1098  
1099  
1099  
1100  
1101  
1102  
1103  
1104  
1105  
1106  
1107  
1108  
1109  
1109  
1110  
1111  
1112  
1113  
1114  
1115  
1116  
1117  
1118  
1119  
1119  
1120  
1121  
1122  
1123  
1124  
1125  
1126  
1127  
1128  
1129  
1129  
1130  
1131  
1132  
1133  
1134  
1135  
1136  
1137  
1138  
1139  
1139  
1140  
1141  
1142  
1143  
1144  
1145  
1146  
1147  
1148  
1149  
1149  
1150  
1151  
1152  
1153  
1154  
1155  
1156  
1157  
1158  
1159  
1159  
1160  
1161  
1162  
1163  
1164  
1165  
1166  
1167  
1168  
1169  
1169  
1170  
1171  
1172  
1173  
1174  
1175  
1176  
1177  
1178  
1178  
1179  
1179  
1180  
1181  
1182  
1183  
1184  
1185  
1186  
1187  
1188  
1189  
1189  
1190  
1191  
1192  
1193  
1194  
1195  
1196  
1197  
1197  
1198  
1199  
1199  
1200  
1201  
1202  
1203  
1204  
1205  
1206  
1207  
1208  
1209  
1209  
1210  
1211  
1212  
1213  
1214  
1215  
1216  
1217  
1218  
1219  
1219  
1220  
1221  
1222  
1223  
1224  
1225  
1226  
1227  
1228  
1229  
1229  
1230  
1231  
1232  
1233  
1234  
1235  
1236  
1237  
1238  
1239  
1239  
1240  
1241  
1242  
1243  
1244  
1245  
1246  
1247  
1248  
1249  
1249  
1250  
1251  
1252  
1253  
1254  
1255  
1256  
1257  
1258  
1259  
1259  
1260  
1261  
1262  
1263  
1264  
1265  
1266  
1267  
1268  
1269  
1269  
1270  
1271  
1272  
1273  
1274  
1275  
1276  
1277  
1278  
1278  
1279  
1279  
1280  
1281  
1282  
1283  
1284  
1285  
1286  
1287  
1288  
1289  
1289  
1290  
1291  
1292  
1293  
1294  
1295  
1296  
1297  
1297  
1298  
1299  
1299  
1300  
1301  
1302  
1303  
1304  
1305  
1306  
1307  
1308  
1309  
1309  
1310  
1311  
1312  
1313  
1314  
1315  
1316  
1317  
1318  
1319  
1319  
1320  
1321  
1322  
1323  
1324  
1325  
1326  
1327  
1328  
1329  
1329  
1330  
1331  
1332  
1333  
1334  
1335  
1336  
1337  
1338  
1339  
1339  
1340  
1341  
1342  
1343  
1344  
1345  
1346  
1347  
1348  
1349  
1349  
1350  
1351  
1352  
1353  
1354  
1355  
1356  
1357  
1358  
1359  
1359  
1360  
1361  
1362  
1363  
1364  
1365  
1366  
1367  
1368  
1369  
1369  
1370  
1371  
1372  
1373  
1374  
1375  
1376  
1377  
1378  
1378  
1379  
1379  
1380  
1381  
1382  
1383  
1384  
1385  
1386  
1387  
1388  
1389  
1389  
1390  
1391  
1392  
1393  
1394  
1395  
1396  
1397  
1397  
1398  
1399  
1399  
1400  
1401  
1402  
1403  
1404  
1405  
1406  
1407  
1408  
1409  
1409  
1410  
1411  
1412  
1413  
1414  
1415  
1416  
1417  
1418  
1419  
1419  
1420  
1421  
1422  
1423  
1424  
1425  
1426  
1427  
1428  
1429  
1429  
1430  
1431  
1432  
1433  
1434  
1435  
1436  
1437  
1438  
1439  
1439  
1440  
1441  
1442  
1443  
1444  
1445  
1446  
1447  
1448  
1449  
1449  
1450  
1451  
1452  
1453  
1454  
1455  
1456  
1457  
1458  
1459  
1459  
1460  
1461  
1462  
1463  
1464  
1465  
1466  
1467  
1468  
1469  
1469  
1470  
1471  
1472  
1473  
1474  
1475  
1476  
1477  
1478  
1478  
1479  
1479  
1480  
1481  
1482  
1483  
1484  
1485  
1486  
1487  
1488  
1489  
1489  
1490  
1491  
1492  
1493  
1494  
1495  
1496  
1497  
1497  
1498  
1499  
1499  
1500  
1501  
1502  
1503  
1504  
1505  
1506  
1507  
1508  
1509  
1509  
1510  
1511  
1512  
1513  
1514  
1515  
1516  
1517  
1518  
1519  
1519  
1520  
1521  
1522  
1523  
1524  
1525  
1526  
1527  
1528  
1529  
1529  
1530  
1531  
1532  
1533  
1534  
1535  
1536  
1537  
1538  
1539  
1539  
1540  
1541  
1542  
1543  
1544  
1545  
1546  
1547  
1548  
1549  
1549  
1550  
1551  
1552  
1553  
1554  
1555  
1556  
1557  
1558  
1559  
1559  
1560  
1561  
1562  
1563  
1564  
1565  
1566  
1567  
1568  
1569  
1569  
1570  
1571  
1572  
1573  
1574  
1575  
1576  
1577  
1578  
1578  
1579  
1579  
1580  
1581  
1582  
1583  
1584  
1585  
1586  
1587  
1588  
1589  
1589  
1590  
1591  
1592  
1593  
1594<br

halftone quality, and moreover excellent in the storage stability.

We claim:

1. A photographic material comprising a light-sensitive silver halide emulsion layer coated on a support which material contains a combination of a salt of tetrazolium containing only a non-metallic anion and a salt of tetrazolium containing a metallic anion, said metallic anion being a complex salt of an organic multivalent aminomultivalent carboxylic acid with a metal selected from the group consisting of iron, cobalt, nickel, copper, lead, chromium, titanium, cerium, samarium, europium and ytterbium, the valency of said metal ions being divalent for copper, trivalent for iron, cobalt, nickel, samarium, europium, chromium and ytterbium, and tetravalent for titanium, cerium, and lead in at least one of said silver halide emulsion layer or in a hydrophilic colloid layer adjacent to said silver halide emulsion layer.

2. A photographic material as claimed in claim 1 wherein the metallic anion is an iron (III), cobalt (III) or nickel (III) complex salt of an organic multivalent amino-multivalent carboxylic acid.

3. A photographic material as claimed in claim 1 wherein the salt of tetrazolium containing only a non-metallic anion is represented by the following Formula (I):  $[T^n\oplus][X_1\ominus]_n$ , in which T represents a tetrazolium cation,  $X_1$  represents an anion containing only non-metallic atoms, and n is an integer of 1 or 2.

4. A photographic material as claimed in claim 1 wherein said salt of tetrazolium containing only a non-metallic anion and said salt of tetrazolium containing a metallic anion are in the silver halide emulsion layer.

5. A photographic material as claimed in claim 1 or 4 wherein said salt of tetrazolium containing only a non-metallic anion and said salt of tetrazolium containing a

metallic anion are each in an amount of  $10^{-5}$ - $10$  mol per 1 mol silver halide.

6. A photographic material as claimed in claim 3 wherein T consisting in Formula (I) represents triphenyltetrazolium and  $X_1$  represents an alkylsuccinic acid ester sulfonate.

7. A photographic material as claimed in claim 2 wherein the metallic anion is an iron (III) complex salt of an organic multivalent amino-multivalent carboxylic acid.

8. A process for developing a photographic material comprising a light-sensitive silver halide emulsion layer coated on a support which material contains a combination of a salt of tetrazolium containing only a non-metallic anion and a salt of tetrazolium containing a metallic anion, said metallic anion being a complex salt of an organic multivalent aminomultivalent carboxylic acid with a metal selected from the group consisting of iron, cobalt, nickel, copper, lead, chromium, titanium, cerium, samarium, europium and ytterbium, the valency of said metal ions being divalent for copper, trivalent for iron, cobalt, nickel, samarium, europium, chromium and ytterbium, and tetravalent for titanium, cerium, and lead in at least one of said silver halide emulsion layer or in a hydrophilic colloid layer adjacent to said silver halide emulsion layer; said process comprising

image-wise exposing said photographic material and then developing said photographic material with a developer containing from 5 to 300 g/liter of a sulfite.

9. The process of claim 8 wherein said photographic material is developed with a developing solution containing p-methylaminophenol sulfate or 1-phenyl-3-pyrazolidone-hydroquinone or mixtures thereof.

10. The process of claim 8 or 9 wherein said developer also contains from 5 to 300 g/liter of a carbonate.

\* \* \* \* \*

UNITED STATES PATENT AND TRADEMARK OFFICE  
CERTIFICATE OF CORRECTION

PATENT NO. : 4,318,979

Page 1 of 2

DATED : March 9, 1982

INVENTOR(S) : TAKESHI HABU et al

It is certified that error appears in the above-identified patent and that said Letters Patent is hereby corrected as shown below:

Column 9, in the last formula appearing at bottom of column,  
that portion of the formula reading " Z " should read



Column 10, line 27: "COO<sup>63</sup>" should be --COO<sup>Θ</sup>--.

Column 10, line 28: "[T<sup>61</sup>]" should be --[T<sup>⊕</sup>]--.

Column 14, line 60: "balck" should be --black--.

Column 16, line 64; "balckened" should be --blackened--.

Columns 17 and 18, TABLE 1: 4th column, 4th line, "II-5"  
should be -- II-2/II-5 --; 7th column, 8th line, "0.07"  
should be --0.04--; 11th column, 6th line, "6.3" should  
be --6.5--; 12th column, penultimate line, "103" should  
be --105--; 15th column, 6th and 7th lines, "95" should  
be --98--, and penultimate line, "103" should be --105--;  
last column, 6th line, "6.3" should be --6.5--.

UNITED STATES PATENT AND TRADEMARK OFFICE  
CERTIFICATE OF CORRECTION

PATENT NO. : 4,318,979

Page 2 of 2

DATED : March 9, 1982

INVENTOR(S) : TAKESHI HABU et al

It is certified that error appears in the above-identified patent and that said Letters Patent is hereby corrected as shown below:

Column 17, line 46: "reslts" should be --results--.

Columns 19 and 20, TABLE 3: 7th column, 4th line, the value "3 x 13<sup>-3</sup>" should be -- 3 x 10<sup>-3</sup> --.

Signed and Sealed this

Second Day of November 1982

[SEAL]

*Attest:*

GERALD J. MOSSINGHOFF

*Attesting Officer*

*Commissioner of Patents and Trademarks*